

## UNITED STATES PATENT OFFICE.

KURT WOETZEL, OF KOBE, JAPAN, AND HEINRICH LINT, OF OFFENBACH-ON-THE-MAIN, GERMANY, ASSIGNORS TO I. G. FARBENINDUSTRIE AKTIENGESELLSCHAFT, OF FRANKFORT, GERMANY.

## PRODUCTION OF AZODYESTUFFS ON SILK.

No Drawing. Application filed November 9, 1925, Serial No. 67,9191, and in Germany June 20, 1925.

Our invention relates to the production of azodyestuffs on natural silk consisting in impregnating the silk fiber with a solution of an azocomponent having a substantive character 5 and developing with a diazo solution.

The fabrics, dyed in this manner, also form a part of the present invention.

The production of ice colors on natural silk is made possible by using azocomponents having a substantive character. As such compounds the arylides of hydroxynaphthoic acids and bodies containing a methylene group capable of combining may be named, such as for example the di- and monoacylacetarylides described in the U. S. Patents Nos. 1,594,864; 1,580,709; 1,594,866, and 1,594,867.

The process of producing ice colors on silk can be executed by impregnating the boiled off silk fiber, preferably at a low temperature (20-30° C.) and while using a protective colloid, with the alkaline solutions of the azocomponents having a substantive character and by developing with diazo solutions, with 5 the surprising result that the quality of the silk fiber with regard to stability, brightness and touch is not affected.

But the azodyestuffs can be produced in the same manner on raw silk which has not been boiled off previously. Such raw silk may be boiled off and bleached with hydrogen peroxide after the dyeing operation. Any undyed raw silk or cotton present and boiled off at the same time, will not affect the dyed silk nor does the latter stain such undyed materials.

Finally the impregnation and boiling off of the raw silk may also be executed in the same operation of manufacture and the development with a diazo solution afterwards.

The process may be used also for silk in mixed woven fabrics.

In this manner fast and brilliant dyeings on silk can be obtained in a simple process of dyeing instead of the hitherto existing expensive and complicated procedures. This result could not be foreseen, because beta naphthol is known to be not adapted for producing ice colors on silk.

The following examples illustrate our invention:

## Example 1.

The boiled off silk or chappe is impregnated for about 20-25 minutes at 25-30° C. with a solution containing 1 gr. of beta-naphthalid of 2,3-hydroxy naphthoic acid in the liter, then 10 p. c. of common salt of the weight of the goods are added and the goods are handled for also 20 minutes, centrifuged thoroughly, then developed for 10-15 minutes with a solution containing 2.3 gr. of diazotised 4-nitro-2-anisidin in the liter, feebly acidulated with hydrochloric acid, well rinsed and twice soaped for about 15-20 minutes with a nearly boiling solution, containing 4-5 gr. of marseilles soap in the liter, rinsed in a warm and cold state and passed by a bath containing acetic or formic or sulfuric or tartaric acid and dried in a not too hot condition. The used beta-naphthalid of 2,3-hydroxy naphthoic acid was dissolved in the triple quantity of caustic soda solution of 34° Bé. after addition of the double quantity of Turkey red oil. To the impregnating bath we then added, as a protective colloid, 1 gr. of "protectol I double powder," a purified cellulose lye, which, as is well-known to those skilled in the art, will protect silk fibres during washing and dyeing, particularly in the presence of alkalies. In this manner a scarlet red shade of an excellent fastness is obtained. The resulting product may be represented by the formula:



## Example 2.

The raw silk is impregnated for about 20 to 25 minutes at from 25 to 30° C. with a solution containing 1.5 gr. of diaceto acetyl-

100

ortho-tolidin in the liter and developed with a solution containing 1.65 gr. of diazotised ortho-chloroanilin in the liter, feebly acidulated with hydrochloric acid, well rinsed and 5 then boiled off for an hour in a nearly boiling bath, containing 30 p. c. of Marseilles soap, together with undyed raw silk and cot-

tives of the 2,3-hydroxy naphthoic acid and other bodies containing a methylene group capable of combining and other azo components having a substantive character may be used for impregnating and other diazo compounds for developing. The resulting product may be represented by the formula: 70



ton, then repassed in a second soaping bath containing 10-15 p. c. of Marseilles soap for 20 completely removing the bast and worked up, as described in Example 1. A brilliant yellow is obtained, which neither is diminished in tone by the additional boiling off nor stains the undyed raw silk and cotton, boiled 25 off at the same time. The resulting product may be represented by the formula: 90



*Example 3.*

The raw silk is impregnated for about 20-25 minutes at 40-60° C. with a solution containing 1 gr. of di-2,3-hydroxy naphthoyl dianisidin in the liter, being boiled off simultaneously by the higher temperature of the bath, then the bath is cooled down to 30° C., 10 p. c. of common salt of the weight of the silk are added and the goods are handled for further 20 minutes, centrifuged thoroughly, 45 then developed for 10 minutes with a solution containing 1.75 gr. of diazotised 5-nitro-2-anisidin in the liter, feebly acidulated with hydrochloric acid, well rinsed and then soaped for half an hour in a nearly boiling bath, containing 15 p. c. of Marseilles soap, for completely developing the color and for completely removing the bast, and worked up as described in Example 1. The used di-2,3-hydroxy naphthoyl-dianisidin was dissolved with the triple quantity of caustic soda 55 solution of 34° Bé. and the double quantity of Turkey red oil. Then such a quantity of caustic soda solution was added to the impregnating bath, that the total quantity was 60 6 gr. of NaOH in the liter of the impregnating bath. As protective colloid 4.5 gr. of "protectol I double powder" was added for each liter of the impregnating bath, a beautiful claret of an excellent fastness is obtained. In the same manner other deriva- 65

Now what we claim, is:

1. The production of azodyestuffs on natural silk consisting in impregnating the silk fiber with a solution of an arylide of 2,3-hydroxy naphthoic acid and in developing with a diazo solution. 85

2. Natural silk materials, dyed according to the process of claim 1. 90

In testimony, that we claim the foregoing as our invention, we have signed our names, this 18th day of August, 1925 (by HEINRICH LINT) and this 26th day of September, 1925 (by KURT WOETZEL). 95

KURT WOETZEL.  
HEINRICH LINT.

100

105

110

115

120

125

130